

[54] TITANIUM BETA S-ALLOY

[75] Inventors: Mary F. Schuler, Virginia Beach, Va.; Ernest P. Abrahamson, Waltham, Mass.

[73] Assignee: The United States of America as represented by the Secretary of the Army, Washington, D.C.

[22] Filed: Oct. 27, 1971

[21] Appl. No.: 190,455

[52] U.S. Cl..... 148/32.5, 75/175.5, 148/12.7

[51] Int. Cl..... C22c 15/00, C22f 1/18

[58] Field of Search..... 75/175.5, 11.5, 148/12.7, 32, 32.5, 133

[56] References Cited

UNITED STATES PATENTS

3,269,825 8/1966 Vordahl..... 75/175.5 X

OTHER PUBLICATIONS

Alloy Digest, Filing Code Ti-59, July 1970, Engineering Alloy Digest Inc., N.J.

Primary Examiner—Charles N. Lovell  
Attorney—Harry M. Saragovitz et al.

[57] ABSTRACT

An improved titanium beta alloy and method for the preparation thereof consisting of the following components in the percent by weight indicated: 10.0 – 12.0% molybdenum; 4.0 – 6.0% zirconium; 3.5 – 5.5% tin; 0.4 – 1.5% tantalum; 0.2 – 1.2% columbium, and the remainder titanium.

2 Claims, No Drawings

## TITANIUM BETA S-ALLOY

The invention described herein may be manufactured, used, and licensed by or for the Government for governmental purposes without the payment to us of any royalty thereon.

This invention relates to a titanium beta alloy comprising an ultra fine grain composition thereby resulting in improved strength characteristics.

A titanium alloy known as Titanium Beta III is commercially available. The alloy comprises, e.g., the following components in the percent by weight indicated: 11.0% molybdenum; 6.0% zirconium; 4.5% tin and 78.5% titanium. In addition to the above components, the present titanium beta S-alloy comprises small amounts of transition metal solutes, i.e., tantalum and columbium. The present alloy has been designated an "S" alloy in order to distinguish it over other alloys. The inclusion of the transition metal solutes serves to raise the recrystallization temperature during fabrication, i.e., forging or rolling of the alloy at a temperature of about 1350°- 1400°F. Raising the recrystallization temperature allows a higher temperature of deformation and hence greater ease of deformation. At the same time, higher recrystallization temperatures inhibits grain growth which allows formation of a submicron grain size. For optimum properties, the fabricated alloy is subsequently heat treated at a temperature of about 900°F for a period of about 8 hours in ambient air.

It is an object of this invention to provide and disclose an improved titanium beta alloy.

It is a further object of this invention to provide and disclose a titanium beta alloy having improved yield and tensile strength characteristic.

It is a further object of this invention to provide and disclose a titanium beta alloy having improved ductility characteristics.

It is a further object of this invention to provide and disclose a titanium beta alloy having improved hardness characteristics.

It is a further object of this invention to provide and disclose a method for the production of an improved titanium beta alloy.

An exemplary composition of the alloy was prepared utilizing about 1 lb. of a mixture consisting of the following components in the percent by weight indicated: 78.15% Ti; 11.0% Mo; 5.0% Zr; 4.5% Sn; 1.0% Ta and 5 0.35 Cb. A range of 10.0 - 12.0% Mo; 4.0 - 6.0% Zr; 3.5 - 5.5% Sn; 0.4 - 1.5% Ta; 0.2 - 1.2% Cb and the remainder Ti has been found operable. The mixture was placed into a water-cooled copper crucible and the crucible positioned into a conventional electric furnace

10 equipped with tungsten electrodes for arc melting. The mixture was melted, cooled and subsequently remelted two more times in order to insure homogeneity. The resultant ingot had a grain size of about one millimeter to about one centimeter.

15 The ingot is recovered from the crucible and forged at a temperature of about 1350°- 1400°F. In lieu of forging, the ingot may be rolled. The fabrication, i.e., forging or rolling, is continued until a minimum breakdown of the material of at least 4 to 1 is achieved, e.g., the reduction of an ingot having a thickness of about 4 inches to a thickness of about 1 inch. The fabricated material is subsequently cooled in ambient air to room temperature.

20 25 Tensile specimens were machined from forged  $\frac{1}{2}$  inch diameter bars. Certain of the bars were heated for a period of 8 hours at a temperature of about 900°F. The objective of the heat treatment is to effect or accelerate the precipitation and agglomeration of the constituents held in supersaturated solid solution. This treatment is called "ageing" or "age-hardening."

30 35 Metallographic examination of the microstructure of the fabricated alloy at a magnification of 1500X has indicated that the grain size developed in the present alloy is in the range of 1 micron or less. This was confirmed by an electron transmission study which established a grain size of 0.9 microns.

40 The tensile specimens, i.e., forged and age-hardened, 40 were subjected to mechanical tests to evaluate their mechanical properties. Composite results consisting of the average of about 10 individual evaluations of tensile specimens are set forth in Table I below.

TABLE I

|             | Yield strength<br>Ksi (0.2 percent) | Tensile strength<br>Ksi | Percent elongation | Percent reduction in area | Hardness Rc |
|-------------|-------------------------------------|-------------------------|--------------------|---------------------------|-------------|
| 1 As forged | —                                   | 117.6                   | 181.9              | 5.23                      | 15.5        |
| 2 900°F     | 8                                   | 258.4                   | 259.7              | 3.9                       | 6.5         |

Other objects and a fuller understanding of the invention may be ascertained from the following description and claims.

55 Available data in regards to the mechanical characteristics of commercially available titanium beta III is set forth in Table II below.

TABLE II

| Rod diameter<br>(inch) | Aging temp. °F | Time<br>(hours) | Yield strength<br>Ksi (0.2 percent) | Tensile strength<br>(Ksi) | Percent elongation | Percent reduction in area |
|------------------------|----------------|-----------------|-------------------------------------|---------------------------|--------------------|---------------------------|
| 1 0.500                | as hot rolled. | —               | 108.4                               | 121.1                     | 26.0               | 80.1                      |
| 2 0.316                | 900            | 8               | 180.8                               | 197.7                     | 10.0               | 19.6                      |
| 3 0.500                | 900            | 8               | 187.6                               | 199.5                     | 9.62               | 27.25                     |
| 4 0.522                | 900            | 8               | 191.0                               | 201.0                     | 11.0               | 33.0                      |

The present titanium alloy exhibits significant improvement in yield and tensile strength over the prior art titanium beta III alloy. The present alloy in the "as forged" condition exhibits improvements in the range of about 60 percent yield strength and about 65 percent tensile strength. Preliminary heat treating studies have shown an improvement of about 70-75 percent yield strength and about 75-80 percent in tensile strength of the present alloy over the prior art alloy. In general, the development of high strength materials of the present invention results in reduced ductility as shown in Table I. However, materials of fine grain size exhibit improved ductility in comparison with materials of coarse grain size at identical yield strength level.

A prior art heat treated titanium beta III tensile specimen was examined for grain size and tested for hardness. The grain size was in the range of 2-3 microns. This compares with a grain size of less than 1 micron for the present alloy. In addition, the hardness of the prior art alloy was Rc 35 compared with a hardness of Rc 48 for the present alloy.

Presently, considerable interest is focused on the development of high strength-to-density ratio titanium alloy because of military requirements for aircraft, armor and structural applications. However, the present titanium alloy could be advantageously utilized in any structure requiring a material having a high strength-to-density ratio.

Although we have described our invention with a certain of particularity it is understood that the present

disclosure has been made only by way of example and that numerous changes may be made in the preparation and fabrication of the present alloy without departing from the spirit and scope of the invention.

Having described our invention, we claim:

1. A wrought age-hardened titanium beta S-alloy product having a fine grain size in the range of 1 micron or less and consisting of the following components in the percent by weight indicated:

|    |           |
|----|-----------|
| Mo | 10.0-12.0 |
| Zr | 4.0-6.0   |
| Sn | 3.5-5.5   |
| Ta | 0.4-1.5   |
| Cb | 0.2-1.2   |

and the remainder titanium, said product having been reduced during fabrication until a minimum breakdown of material of at least 4 to 1 is achieved.

2. A titanium beta S-alloy product in accordance with claim 1 consisting essentially of the following components in the percent by weight indicated:

|    |       |
|----|-------|
| Mo | 11.0  |
| Zr | 5.0   |
| Sn | 4.5   |
| Ta | 1.0   |
| Cb | 0.35  |
| Ti | 78.15 |

\* \* \* \* \*